

(No Model.)

D. G. FITZ-GERALD.

OBTAINING CHLORINE BY ELECTROLYSIS.

No. 357,659.

Patented Feb 15, 1887.



Attest.  
Willet Norton.  
W. F. Huntzemann

Inventor.  
Desmond G. Fitzgerald  
by John F. Haleed & Son  
his Atts.

# UNITED STATES PATENT OFFICE.

DESMOND GERALD FITZ-GERALD, OF AKERMAN ROAD, LOUGHBOROUGH ROAD, BRIXTON, COUNTY OF SURREY, ENGLAND.

## OBTAINING CHLORINE BY ELECTROLYSIS.

SPECIFICATION forming part of Letters Patent No. 357,659, dated February 15, 1887.

Application filed October 18, 1886. Serial No. 216,602. (No model.)

*To all whom it may concern:*

Be it known that I, DESMOND GERALD FITZ-GERALD, a subject of the Queen of Great Britain, residing at 6 Akerman Road, Loughborough Road, Brixton, in the county of Surrey, England, electrician, have invented certain new and useful Improved Means for Effecting the Electro-Chemical Generation of Chlorine in Metallurgical Operations for the Extraction of Gold from its Ores and for other Purposes, of which the following is a specification.

The great difficulty in the electrolytic generation of chlorine by the decomposition under the influence of an electric current of hydrochloric acid or of an alkaline or earthy chloride in solution has been to find a suitable anode unacted upon by the gas in its nascent condition. One material only—viz., carbon, usually in the form known as "gas carbon"—has hitherto been available for use on a large scale in the above operation. This material, however, is far from fulfilling the condition of being unacted upon chemically and mechanically by the evolved chlorine. The ultimate disintegration of the carbon anode, together with the difficulty of establishing efficient electrical contact between fragments or plates of this material, has led to the failure in practice of electrolytic processes for the extraction of the precious metals from their ores by means of chlorine and for the utilization of this element in various other directions.

Now, I have found that peroxide of lead in the form of dense conductive plates, layers, or masses answers admirably the purpose of an anode for the electrolytic generation of chlorine. Being already in the highest condition of oxidation, it is not liable to further action in this direction, nor is it acted upon by the hypochlorites, or liable to disintegration by the effect of the nascent chlorine evolved from its surface. The only precaution I have in any case found necessary to insure the permanency of such plates, layers, or masses when employed as anodes is, when free hydrochloric acid is contained in the electrolyte, to avoid the prolonged contact of the peroxide with this acid when the current is no longer passing.

In the accompanying drawing, in section,

A A is a tank of slate or of brick lined with suitable material; B B, anode of lead peroxide; C, contact-piece of platinum; D D, cathode of copper forming a tray, of which the outer surface is coated with insulating material; E, ore to be acted upon by chlorine; F, electrolyte.

In carrying my invention into effect for the purpose of extracting gold from its ores and for other metallurgical purposes, I usually construct anodes of large surface, applied to and supported by a portion of the interior surface of an electrolytic tank in such manner that the ore to be treated may be in contact with the anode surface, and may thus be permeated by the evolved chlorine when the anode is used for the required purpose. In any case I employ in the construction of the anode a plastic composition of oxide of lead (or of an equivalent insoluble compound of lead susceptible, like the oxide, of being subsequently converted into peroxide of lead by electrolytic action) in admixture with a solution—such as that of the sulphate or chloride of ammonium—which will more or less gradually and partially react upon the lead compound to produce a chemical change, causing the composition to "set" and to acquire a high degree of solidity. I thus avoid any admixture with the lead compound of inert material—such as plaster-of-paris or other cement—which would render impossible the ultimate production of a highly-conductive mass of peroxide of lead. I have constructed anodes wholly of this composition, applied by means of a trowel, while yet freshly mixed, to a portion of the interior surface (as shown in the accompanying figure) of an electrolytic tank; but by reason of the effects sometimes produced by the very considerable expansion which occurs during its conversion into peroxide I prefer to employ this composition merely as a kind of mortar, by means of which I build up the anode by uniting together slabs, plates, fragments, or granules of peroxide of lead, or of an insoluble compound of lead more or less superficially converted into peroxide of lead.

The course I usually adopt, therefore, in the construction of anodes of large surface is, first, to produce slabs, plates, "tiles," or granules of the compositions hereinabove described, 100

by compressing in suitable molds the freshly-mixed plastic mass composed of oxide of lead (litharge) with (for instance) a half-saturated solution of sulphate of ammonia, or with a solution of hydropotassic sulphate (sal-enixum) or hydrosodic sulphate, or by passing it through a sieve or granulating-machine; secondly, to superficially convert the slabs, plates, or granules, when set or hardened, into peroxide of lead by the action of a hot solution of an alkaline or earthy hypochlorite; thirdly, to build up the anode upon a suitable supporting-surface, using for this purpose as a mortar or cement the aforesaid plastic material in a freshly-mixed condition; and, lastly, to effect a further conversion of the material into peroxide of lead by the passage of a current through the mass when it has obtained a sufficient degree of hardness and solidity. In effecting the electrolytic conversion last mentioned, I prefer to employ as the electrolyte dilute sulphuric acid or a solution of the sulphate of soda or of magnesia. Contact with the anode material may be obtained by means of a plate of platinum embedded in the upper portion of the mass, and any suitable cathode—such as a plate of copper—may be employed to complete the circuit of the dynamo-machine or other source of electricity used to effect the conversion of the material into peroxide. When this conversion has been effected to a sufficient extent—*i. e.*, when the whole surface of the anode has acquired a dark-brown color, and evolves in lieu of absorbing the oxygen liberated by the passage of the current—the above-mentioned electrolyte may be replaced by the chloride solution to be employed in the generation of chlorine.

I have given as an example one mode in which peroxide of lead may be utilized, according to my invention, for the electro-chemical generation of chlorine on a large scale, and I have indicated the only known means, so far as I am aware, by which indestructible anodes of this material—that is, slabs, plates, or masses not liable to disintegration—not in contact with any oxidizable (conducting) support,

and possessing a sufficiently high degree of conductivity to allow of the conducting support being dispensed with, may be readily obtained; but I do not confine myself to the above-described mode of utilizing peroxide of lead as an anode which is convenient and effective in the treatment of ores or compounds containing gold; nor do I limit myself to the precise modes of obtaining peroxide of lead in a coherent form, which have been referred to. It is obvious that in the electro-chemical generation of chlorine for bleaching purposes, or for the manufacture of hypochlorites or of chlorates, a series of vertically-disposed plates of peroxide of lead alternating with cathode-plates of any suitable conducting material may conveniently be employed, and it is possible to obtain such plates by various means, which, according to my experience, are less convenient and effective than those which have been indicated above. Again, it is not essential in all cases to obtain contact with the peroxide by means of platinum. For instance, the vertically-disposed plates just mentioned may be connected together and with an external conductor by means of an alloy fusible at a comparatively low temperature, such alloy being subsequently protected from electro-chemical action by means of a layer of cement.

What I claim as my invention is—

The electro-chemical generation of chlorine by means of an anode of peroxide of lead in the form of dense highly-conductive layers, plates, or masses of any required form, preferably obtained by the means hereinbefore described, the said anode being employed in conjunction with any suitable cathode and with an electrolyte capable of evolving chlorine. 85

In testimony whereof I, the said DESMOND GERALD FITZ-GERALD, have hereunto set my hand this 12th day of August, 1886.

DESMOND GERALD FITZ-GERALD.

Witnesses:

G. F. WARREN,

*Notary Public,*

WALTER J. SKERTEN,  
Both of 17 Gracechurch St., London.